

# UNITED STATES PATENT OFFICE.

HERBERT M. SMITH, OF GREAT BARRINGTON, MASSACHUSETTS, ASSIGNOR TO STANLEY INSULATING COMPANY, OF GREAT BARRINGTON, MASSACHUSETTS, A CORPORATION OF MAINE.

## METHOD OF PRODUCING AND APPLYING ENAMEL COATINGS TO METALLIC SURFACES.

1,425,612.

Specification of Letters Patent. Patented Aug. 15, 1922.

No Drawing.

Application filed September 30, 1918. Serial No. 256,283.

To all whom it may concern:

Be it known that I, HERBERT MILLS SMITH, a citizen of the United States, residing at Great Barrington, in the county of 5 Berkshire and State of Massachusetts, have invented certain new and useful Improvements in Methods of Producing and Applying Enamel Coatings to Metallic Surfaces, of which the following is a specification.

10 This invention relates to a method of producing and applying a vitreous enamel for insulated containers and receptacles and that will stand mechanical shock, rapid thermal changes and deflection. With this 15 object in view I have produced a new combination of materials, have devised a novel and effective way of preparing the metallic surface to which it is to be applied, and have provided for the removal, as rapidly as they 20 are formed, of the gases which are formed during the fusion of the enamel.

Other objects of the invention, more or less broad than those stated above, together with the advantages inherent, will appear 25 from the following description of the elements, combinations, arrangements of parts and applications of principles constituting the invention; and the scope of protection contemplated will appear from the claims.

30 Assuming that the surface to which the enamel is to be applied is a metal like steel, the first step is to heat the receptacle so as to consume and drive off any organic or greasy coating which may be on the metal. 35 As the next step I remove the metallic oxides, as by any suitable electrolytic process. Since such electrolytic process ordinarily involves the use of an acid electrolyte, all trace of acid must be removed from. 40 the metal. This I accomplish by first washing the surface in water and then in a solution which will neutralize any remaining acid.

The result is that I have a metal with an 45 eggshell matte surface or finish to which the enamel coat will most effectively adhere.

The enamel consists of two distinct combinations of materials. One is called the ground coat and consists of the following

materials in about the amounts and proportions stated:

|                    | Amount.    | Per cent. |
|--------------------|------------|-----------|
| Feldspar           | 36.00 lbs. | 23.74     |
| Quartz             | 33.00 "    | 21.76     |
| Borax              | 50.20 "    | 33.11 55  |
| Soda nitrate       | 10.70 "    | 7.04      |
| Salt peter         | 6.50 "     | 4.28      |
| Clay               | 6.00 "     | 3.95      |
| Fluorspar          | 6.30 "     | 4.15      |
| Epsom salts        | .19 "      | .13 60    |
| Cobalt oxide       | .25 "      | .18       |
| Nickel oxide       | .30 "      | .21       |
| Copper oxide       | .50 "      | .35       |
| Magnesia carbonate | 1.20 "     | .80       |
| Manganese dioxide  | .46 "      | .30 65    |
|                    | 151.60 "   |           |

The above materials are mixed and fused to make a frit, being afterwards ground up and then mixed with a small quantity of 70 water to form a mass of about the consistency of thick cream.

The cover coat contains the following materials in about the amounts and proportions stated, and these materials are mixed 75 and fused just as are the materials for the ground coat:

|                    | Amount.    | Per cent. |
|--------------------|------------|-----------|
| Feldspar           | 35.00 lbs. | 22.06 80  |
| Quartz             | 33.00 "    | 20.80     |
| Borax              | 41.20 "    | 25.98     |
| Soda nitrate       | 15.00 "    | 9.46      |
| Cobalt oxide       | 2.13 "     | 1.34      |
| Manganese dioxide  | 1.07 "     | .67       |
| Salt peter         | 4.00 "     | 2.52 85   |
| Magnesia carbonate | 1.18 "     | .74       |
| Clay               | 5.87 "     | 3.70      |
| Fluorspar          | 10.00 "    | 6.31      |
| Epsom salts        | .18 "      | .11       |
| Kryolite           | 10.00 "    | 6.31 90   |
|                    | 158.63 "   |           |

The receptacle properly cleaned as before described is filled with a quantity of the 95 liquid enamel mixture, the ground coat, and shaken so as to distribute the enamel mixture over the surface. Then the receptacle

is emptied and heated so as to dry out the enamel. Next it is put in a furnace heated to about one thousand degrees centigrade and left for approximately three minutes 5 for fusion. While this fusion is going on a blast of hot air is introduced into the interior of the receptacle for the purpose of removing, as fast as they are formed, the gases resulting from the fusion of the various materials which would otherwise result 10 in a bubbled and uneven surface. Incidentally the blast may have the effect of evening the distribution of the fused coating. The receptacle is now removed from the furnace 15 and allowed to cool and then is filled with the second or covering enamel mixture which is applied in the same way as the first or ground coat, and with the air blast as before, but with a temperature reduced to 20 about 800° C. I apply the cover coat at a reduced temperature of fusion so as not to refuse the first coat and cause a commingling of the two and a disturbance of the adhesion of the first coat to the metal surface. The 25 first cover coat having been applied the receptacle is removed from the furnace and cooled and the receptacle is again filed with

the coating mixture and emptied and put into the furnace again as before with the air blast but with a temperature now reduced to about 750° C., thus accomplishing the fusion of the third coat without disturbing either of the previous coats. 30

The result is a vitreous flexible coating 35 evenly distributed and uniform in texture which will stand mechanical shock, rapid thermal changes, and bending or deflection of the walls to which it is applied.

I claim:—

1. As a part of the process of enameling, 40 applying an enamel mixture to a surface which is to be coated thereby, distributing the material over the surface, subjecting it to a fusion temperature and applying an air blast thereto while the fusion is going on. 45

2. As a part of the process of enameling, applying an enamel mixture to a surface distributing the material over the surface, and subjecting the material to a heated air blast to remove the gases resulting from 50 fusion while the fusion is going on.

In testimony whereof I affix my signature in presence of two witnesses.

HERBERT M. SMITH.